

3,657,372

NAPHTHALENE CRYSTAL GROWTH IN A GEL  
John C. Murphy, Ellicott City, and Henry A. Kues, Jr.,  
Carney, Md., assignors to the United States of America  
as represented by the Secretary of the Navy  
No Drawing. Filed Mar. 10, 1969, Ser. No. 805,893  
Int. Cl. B01d 9/02; C07c 15/24  
U.S. Cl. 260—674 A

1 Claim

## ABSTRACT OF THE DISCLOSURE

A method for crystal growth in a diffusion medium is disclosed which utilizes a "co-solute effect" to produce single crystals of a material of interest. Generally, a co-solute is a material soluble in the chosen solvent medium and which increases the solubility in said solvent medium of some material of interest. To practice the invention as taught herein, a co-solute is used which increases the solubility of the material of interest with concentration of the co-solute.

## BACKGROUND OF THE INVENTION

### (A) Field of the invention

The present invention finds utility in the field of crystallization and, more specifically relates to the growth of single crystals by diffusion in organic or inorganic gels.

### (B) Description of the prior art

A number of patents relating to silica gel processes exist. Crystallization from a silica gel is a well-known procedure, having been used for nearly a century.

Growth of single crystals of solid materials requires that the instantaneous supersaturation of the solid phase relative to the dispersed phase be kept at a minimum. This general condition holds for crystal growth from a solvent medium, from a gas or from a melt. Procedures for single crystal growth differ essentially in the manner in which this low supersaturation is maintained. The more obvious differences in growth conditions i.e., temperature, pressure, etc., which distinguish the various methods are determined by the need to satisfy this general condition. For example, simple growth of crystals from aqueous solution is accomplished either by slow evaporation of the solvent or by slow cooling or heating of the solution (depending on whether the solubility-temperature curve is normal or retrograde). In both cases the variation of the external parameter, evaporation rate or temperature, controls the degree of instantaneous supersaturation and hence the rate of precipitation.

The silica gel method of crystal growth, as an example of the general problem of growth in gels, is subject to the above-mentioned condition. To illustrate, a typical prior art silica gel process consists of an addition of an acid to an aqueous solution of sodium metasilicate ( $\text{Na}_2\text{SiO}_3 \cdot 9\text{H}_2\text{O}$ ) or ordinary water glass



To this mixture is added a salt solution containing the X component of the desired crystal form MX. On standing, the solution sets to an elastic gel. After the gel has set, a salt solution containing the M component of the desired crystal form is caused to cover the gel. Crystals of the form MX will appear in the gel usually within a few hours. Of specific importance is the fact that the gel is a permeable medium into which diffusion can occur at room temperature. The rate of diffusion and hence the degree of supersaturation is determined by the density of the gel, the normality of the solutions containing

M and X, and the temperature. Since this diffusion rate can be controlled, low solubility crystals which normally cannot be obtained from ordinary aqueous solution can be grown.

5 Solubility considerations prevent growth of compounds such as mercuric sulfides and silver halides using prior art silica gel methods.

The present invention provides a method which enables the growth of crystals of these compounds while retaining the simplicity and convenience of the silica gel method. Since mercuric sulfide and silver halide crystals are of considerable technological importance, the present method marks a significant advance in the field of crystal production.

## SUMMARY

Growth of single crystals of mercuric sulfides and silver halides is achieved through a modification of the well-known silica gel process. In the above-given description of a typical silica gel process, a solution containing cation M of the desired crystal form MX was added to a prepared gel. In the present method, the desired compound MX is brought into solution through the use of a "co-solute," that is, a material which increases the solubility of the compound MX in either linear or non-linear fashion with concentration of the co-solute. The solution containing the desired compound MX is added to the prepared gel. In the crystal growth operation, the concentration of the combined solution is reduced by diffusion into the gel. As diffusion into the gel of the "ionic partners," M and X occurs, the compound MX crystallizes due to the reduced solubility of the compound MX in the gel environment. The concentration of the co-solute in the gel medium is much less than in the combined solution and, due to the solubility effect, solvation influences are not strong enough to prevent crystallization of the material MX.

At the time of this writing, single crystals of mercuric sulfides and silver halides have been grown by use of the present method utilizing a non-linear solubility dependence. These compounds were previously unobtainable through use of aqueous methods. A number of organic and inorganic materials have been grown in aqueous and non-aqueous solutions using a linear solubility dependence of the material of interest on the co-solute. One example is a solution of naphthalene in acetone which is added to an aqueous gel, the naphthalene forming large single crystals in the gel. The present method, in principle, has general application to crystal growth of related materials.

## DESCRIPTION OF THE PREFERRED EMBODIMENTS

Single crystal growth in a diffusion medium, such as a silica gel, is accomplished by utilizing a "co-solute effect." Generally, a co-solute is a material soluble in the solvent medium in use and which increases the solubility in that medium of some material of interest. To practice the invention as taught herein, a co-solute is used which produces a spatial dispersion of the material of interest in the diffusion medium. The solubility dispersion is effected by one of at least two mechanisms, viz, (1) a non-linear dependence of the solubility of the material of interest on the concentration of the co-solute, and (2) a differential rate of diffusion of the co-solute and the material of interest into the diffusion medium. Both mechanisms may be operable in a particular instance. More generally, the operation of the latter mechanism allows crystallization of compounds having linear solubility dependence on the co-solute.

70 Crystallization of mercuric sulfides and silver halides is achieved in a gel medium by use of a non-linear co-solute effect. The key to the method is the determination

and use of a co-solute which increases the solubility of the material of interest in a non-linear fashion with concentration of the co-solute. Increased solubility of the material of interest is believed due to complex formation in the solution, or to the formation of a soluble double salt.

Small crystals of  $\alpha$ -HgS and  $\beta$ -HgS (~0.5 mm. max.) are grown in silica gel from Na<sub>2</sub>S solution under varied conditions of pH and temperature. In this case, the aqueous solubilities of  $\alpha$ -HgS and  $\beta$ -HgS are known to be enhanced by the presence of Na<sub>2</sub>S. Typically, sodium silicate gels of specific gravity 1.05 in the pH range 5.8-8.5 are formed with nitric acid and allowed to stand overnight. A combined solution of Na<sub>2</sub>S-HgS is added to the top of the gel. In a matter of a day, crystals appear in the gel near the interface and in the solution surmounting the gel. Severe gel shrinkage is evident. Dilution of the original combined solution by the syneresis liquid from the gel is believed to be the principal reason for crystal formation in said solution. Initially, only cubic, black  $\alpha$ -HgS crystals are evident, but on standing for a period of time, conversion to the red hexagonal  $\beta$ -HgS occurs. The rate of conversion and the final size of the HgS crystals increase with temperature in the general range of 20° to 60° C.

Similarly, the solubilities of the various silver halides are known to increase by many orders of magnitude in concentrated alkali halide and alkaline earth halide solutions as well as in silver complex formers such as Na<sub>2</sub>SO<sub>3</sub>, Na<sub>2</sub>S<sub>2</sub>O<sub>3</sub>, and others. The various silver halides are grown from their respective K, NH<sub>4</sub>, Na, O and Ca halide solutions. Typical sizes of the crystals are: AgI~8-10 mm. for all co-solutes; AgBr~3 mm. in NH<sub>4</sub>Br (octahedral), ~2 mm. in KBr (cubic); AgCl~1 mm. in NaCl and CaCl<sub>2</sub> solutions. The procedure employed is as follows. Sodium silicate gels of specific gravity 1.03 are formed in the pH range 5.5-8.5 using acetic acid. After gelling, a concentrated solution of the co-solute to be used, for example KI solution, is added to the top of the gel and allowed to stand for times ranging from one to six days. The co-solute solution is then decanted and the silver halide-co-solute solution, in the case described AgI in KI solution, is substituted in the place of the decanted co-solute solution. Crystals appear within a few hours and grow to the sizes described previously. This procedure greatly suppresses the number of nucleation sites observed without "pre-doping." In the case of the  $\beta$ -AgI crystals, in particular, a number of the crystals had a hexagonal habit with one smooth side, the other side having ridges parallel to the hexagonal sides and radiating from a nucleation site in the center of the plate as has previously been described in the art. A number of crystals grew as triangles~1 cm. on a side with ridges from the apices of the triangle to its center. The remainder of these crystals are perfectly free from other nucleation sites. Optical spectra on these remaining crystals indicate a sharp edge located at 2.85 ev., assuming a direct transition. X-ray results indicate reasonable crystal perfection.

An example of single crystal growth from a gel medium of a material having linear solubility dependence on a co-solute is illustrated by the growth of naphthalene in an aqueous gel where acetone is used as the co-solute. In this particular case, acetone acts not only as the co-solute, but also as the solvent medium for the combined solution. Addition of the naphthalene-acetone solution to an aqueous gel results in the formation of naphthalene crystals in the gel. The operable mechanism in this instance is the differential diffusion rate of the naphthalene and acetone species into the gel. The naphthalene-acetone system additionally illustrates the general nature of the present method, i.e., the use of organic solvents and aqueous gels, etc.

The present method is believed to be general and applicable to a large number of situations and amenable to various conditions of pH, temperature, gel composition, etc. It is believed apparent that the practice of the present method is not limited to the particular description given herein. Variation in concentrations, densities, and materials used are to be expected and permitted within the scope of the appended claim.

What is claimed is:

1. A method for growing single crystals of naphthalene in a sodium silicate gel comprising, preparing in a solvent medium a solution of naphthalene and a co-solute, the co-solute comprising acetone and acting to increase in a linear fashion the solubility of naphthalene in the solvent medium, and introducing the solution into contacting relation with the gel into which the naphthalene exhibits a more rapid rate of diffusion than the rate of diffusion of the co-solute, crystallization of said compound occurring in the gel.

#### References Cited

##### UNITED STATES PATENTS

- |           |         |                        |         |
|-----------|---------|------------------------|---------|
| 2,441,572 | 5/1948  | Hirschler et al. ----- | 208-310 |
| 2,941,018 | 6/1960  | Foreman -----          | 260-674 |
| 3,371,036 | 12/1968 | Torgesen -----         | 23-301  |

##### OTHER REFERENCES

O'Connor et al.: Nature, 212, p. 68 (1966).

Henisch et al.: Crystal Growth In Gels, J. Phys. Chem. Solids, pp. 493-500 (1965).

Strong: Scientific American, March 1962, pp. 155-62.

O'Connor et al.: J. Crystal Growth, 1 (1967), pp. 327-28.

Holmes: Formation of Crystals in Gels, J. Phys. Chem. 21, pp. 714-715 (1917).

NORMAN YUDKOFF, Primary Examiner

R. T. FOSTER, Assistant Examiner

U.S. Cl. X.R.

23-305, 668, 300